



US007709168B2

(12) **United States Patent**  
**Wu et al.**

(10) **Patent No.:** **US 7,709,168 B2**  
(45) **Date of Patent:** **\*May 4, 2010**

(54) **PHOSPHONIUM CONTAINING CHARGE  
TRANSPORT LAYER PHOTOCONDUCTORS**

(75) Inventors: **Jin Wu**, Webster, NY (US); **Edward F Grabowski**, Webster, NY (US); **Kent J Evans**, Lima, NY (US); **Daniel V Levy**, Rochester, NY (US)

(73) Assignee: **Xerox Corporation**, Norwalk, CT (US)

(\*) Notice: Subject to any disclaimer, the term of this patent is extended or adjusted under 35 U.S.C. 154(b) by 328 days.

This patent is subject to a terminal disclaimer.

(21) Appl. No.: **11/869,265**

(22) Filed: **Oct. 9, 2007**

(65) **Prior Publication Data**

US 2009/0092915 A1 Apr. 9, 2009

(51) **Int. Cl.**

**G03G 15/02** (2006.01)

(52) **U.S. Cl.** ..... **430/58.05**; 430/58.35; 430/58.75

(58) **Field of Classification Search** ..... **430/58.75**,  
430/58.05, 58.35

See application file for complete search history.

(56) **References Cited**

U.S. PATENT DOCUMENTS

- |               |         |                               |
|---------------|---------|-------------------------------|
| 4,265,990 A   | 5/1981  | Stolka et al.                 |
| 4,464,450 A   | 8/1984  | Teuscher                      |
| 4,587,189 A   | 5/1986  | Hor et al.                    |
| 4,921,773 A   | 5/1990  | Melnyk et al.                 |
| 5,473,064 A   | 12/1995 | Mayo et al.                   |
| 5,482,811 A   | 1/1996  | Keoshkerian et al.            |
| 5,521,306 A   | 5/1996  | Burt et al.                   |
| 5,882,814 A * | 3/1999  | Fuller et al. ..... 430/58.35 |

6,913,863 B2 7/2005 Wu et al.  
7,037,631 B2 5/2006 Wu et al.  
7,482,103 B2 \* 1/2009 Wu et al. ..... 430/56

OTHER PUBLICATIONS

Jin Wu et al., U.S. Application No. (not yet assigned) on Additive Containing Photogenerating Layer Photoconductors, filed concurrently herewith.

Jin Wu et al., U.S. Application No. (not yet assigned) on Phosphonium Containing Photogenerating Layer Photoconductors, filed concurrently herewith.

Jin Wu et al., U.S. Application No. (not yet assigned) on Additive Containing Charge Transport Layer Photoconductors, filed concurrently herewith.

Jin Wu et al., U.S. Application No. (not yet assigned) on Imidazolium Salt Containing Charge Transport Layer Photoconductors, filed concurrently herewith.

Jin Wu et al., U.S. Application No. (not yet assigned) on Charge Trapping Releaser Containing Charge Transport Layer Photoconductors, filed concurrently herewith.

Jin Wu et al., U.S. Application No. (not yet assigned) on Charge Trapping Releaser Containing Photogenerating Layer Photoconductors, filed concurrently herewith.

Jin Wu et al., U.S. Application No. (not yet assigned) on Salt Additive Containing Photoconductors, filed concurrently herewith.

Liang-Bih Lin et al., U.S. Appl. No. 11/800,108 on Photoconductors, filed May 4, 2007.

Liang-Bih Lin et al., U.S. Appl. No. 11/800,129 on Photoconductors, filed May 4, 2007.

\* cited by examiner

*Primary Examiner*—John L Goodrow

(74) *Attorney, Agent, or Firm*—E. O. Palazzo

(57) **ABSTRACT**

A photoconductor that includes, for example, a supporting substrate, a photogenerating layer, and at least one charge transport layer comprised of at least one charge transport component, and wherein the at least one charge transport layer contains at least one phosphonium salt.

**24 Claims, No Drawings**

## 1

PHOSPHONIUM CONTAINING CHARGE  
TRANSPORT LAYER PHOTOCONDUCTORSCROSS REFERENCE TO RELATED  
APPLICATIONS

U.S. application Ser. No. 11/869,231, U.S. Publication 20090092913, filed Oct. 9, 2007, entitled Additive Containing Photogenerating Layer Photoconductors by Jin Wu et al., the disclosure of which is totally incorporated herein by reference, illustrates a photoconductor comprising a supporting substrate, a photogenerating layer, and at least one charge transport layer comprised of at least one charge transport component, and wherein the photogenerating layer contains at least one of an ammonium salt and an imidazolium salt.

U.S. application Ser. No. 11/869,246, U.S. Publication 20090092914, filed Oct. 9, 2007, entitled Phosphonium Containing Photogenerating Layer Photoconductors by Jin Wu et al., the disclosure of which is totally incorporated herein by reference, illustrates a photoconductor comprising a supporting substrate, a phosphonium salt containing photogenerating layer, and at least one charge transport layer comprised of at least one charge transport component.

U.S. application Ser. No. 11/869,252, U.S. Publication 20090092911, filed Oct. 9, 2007, entitled Additive Containing Charge Transport Layer Photoconductors by Jin Wu et al., the disclosure of which is totally incorporated herein by reference, illustrates a photoconductor comprising a supporting substrate, a photogenerating layer, and at least one charge transport layer comprised of at least one charge transport component, and wherein the charge transport layer contains at least one ammonium salt.

U.S. application Ser. No. 11/869,258, U.S. Publication 20090092912, filed Oct. 9, 2007, entitled Imidazolium Salt Containing Charge Transport Layer Photoconductors by Jin Wu et al., the disclosure of which is totally incorporated herein by reference, illustrates a photoconductor comprising a supporting substrate, a photogenerating layer, and at least one charge transport layer comprised of at least one charge transport component, and wherein at least one charge transport layer contains at least one imidazolium salt.

U.S. application Ser. No. 11/869,269, U.S. Publication 20090092908, filed Oct. 9, 2007, entitled Charge Trapping Releaser Containing Charge Transport Layer Photoconductors by Jin Wu, the disclosure of which is totally incorporated herein by reference, illustrates a photoconductor comprising a supporting substrate, a photogenerating layer, and at least one charge transport layer comprised of at least one charge transport component, and wherein the at least one charge transport layer contains at least one charge trapping releaser.

U.S. application Ser. No. 11/869,279, U.S. Publication 20090092909, filed Oct. 9, 2007, entitled Charge Trapping Releaser Containing Photogenerating Layer Photoconductors by Jin Wu, the disclosure of which is totally incorporated herein by reference, there is disclosed a photoconductor comprising a supporting substrate, a photogenerating layer, and at least one charge transport layer comprised of at least one charge transport component, and wherein the photogenerating layer contains at least one charge trapping releaser component.

U.S. application Ser. No. 11/869,284, U.S. Publication 20090092910, filed Oct. 9, 2007, entitled Salt Additive Containing Photoconductors by Jin Wu, the disclosure of which is totally incorporated herein by reference, illustrates a photoconductor comprising a supporting substrate, a photogenerating layer, and at least one charge transport layer comprised of at least one charge transport component, and wherein at

## 2

least one of the photogenerating layer and the charge transport layer contains at least one of a pyridinium salt and a tetrazolium salt.

In U.S. application Ser. No. 11/800,129, U.S. Publication 20080274419, entitled Photoconductors, filed May 4, 2007 by Liang-Bih Lin et al., the disclosure of which is totally incorporated herein by reference, there is illustrated a photoconductor comprising a supporting substrate, a photogenerating layer, and at least one charge transport layer comprised of at least one charge transport component, and wherein the photogenerating layer contains a bis(pyridyl)alkylene.

In U.S. application Ser. No. 11/800,108, U.S. Publication 20080274418, entitled Photoconductors, filed May 4, 2007 by Jin Wu et al., the disclosure of which is totally incorporated herein by reference, there is disclosed a photoconductor comprising a supporting substrate, a photogenerating layer, and at least one charge transport layer comprised of at least one charge transport component, and wherein the charge transport layer contains a benzoimidazole.

## BACKGROUND

This disclosure is generally directed to imaging members, photoreceptors, photoconductors, and the like. More specifically, the present disclosure is directed to multilayered drum, or flexible, belt imaging members, or devices comprised of a supporting medium like a substrate, a photogenerating layer, and a charge transport layer, including a plurality of charge transport layers, such as a first charge transport layer and a second charge transport layer, and wherein the photogenerating layer contains an additive or dopant, and a photoconductor comprised of a supporting medium like a substrate, a photogenerating layer, and a charge transport layer, including a plurality of charge transport layers, such as a first charge transport layer and a second charge transport layer, and wherein at least one of the charge transport layers contains an additive or dopant.

The additives or dopants which can be incorporated into the charge transport layer or the photogenerating layer, and which dopants function, for example, to passivate the charge transport layer or the photogenerating pigment surface by, for example, blocking or substantially blocking intrinsic free carriers, and preventing or minimizing external free carriers from attracting to the pigment surface, and thereby permitting photoconductors with minimal CDS (charge deficient spots), the control of PIDC, for example controlling, and more specifically, reducing the PIDC, especially in those situations where the photosensitivity of the photoconductor can be adjusted on line and automatically, to a desired preselected value or amount, and which photosensitivity can be increased or decreased; and acceptable LCM characteristics, such as for example, improved lateral charge migration (LCM) resistance.

More specifically, the photoconductors illustrated herein, in embodiments, have excellent wear resistance, extended lifetimes, elimination or minimization of imaging member scratches on the surface layer or layers, such as the charge transport layer of the member, and which scratches can result in undesirable print failures where, for example, the scratches are visible on the final prints generated. Additionally, in embodiments the photoconductors disclosed herein possess excellent, and in a number of instances low  $V_r$  (residual potential), and allow the substantial prevention of  $V_r$  cycle up for at least 10,000 xerographic imaging cycles; low acceptable image ghosting characteristics; low background; and/or minimal charge deficient spots (CDS). At least one in

embodiments refers, for example, to one, to from 1 to about 10, to from 2 to about 7; to from 2 to about 4, to two, and the like.

Also included within the scope of the present disclosure are methods of imaging and printing with the photoconductor devices illustrated herein. These methods generally involve the formation of an electrostatic latent image on the imaging member, followed by developing the image with a toner composition comprised, for example, of thermoplastic resin, colorant such as pigment, charge additive, and surface additives, reference U.S. Pat. Nos. 4,560,635; 4,298,697 and 4,338,390, the disclosures of which are totally incorporated herein by reference, subsequently transferring the image to a suitable substrate, and permanently affixing the image thereto. In those environments wherein the device is to be used in a printing mode, the imaging method involves the same operation with the exception that exposure can be accomplished with a laser device or image bar. More specifically, the imaging members and flexible belts disclosed herein can be selected for the Xerox Corporation iGEN3® machines that generate with some versions over 100 copies per minute. Processes of imaging, especially xerographic imaging and printing, including digital, and/or color printing are thus encompassed by the present disclosure.

The photoconductors disclosed herein are in embodiments sensitive in the wavelength region of, for example, from about 400 to about 900 nanometers, and in particular from about 650 to about 850 nanometers, thus diode lasers can be selected as the light source. Moreover, the imaging members disclosed herein are in embodiments useful in high resolution color xerographic applications, particularly high-speed color copying and printing processes.

#### REFERENCES

There is illustrated in U.S. Pat. No. 6,913,863, the disclosure of which is totally incorporated herein by reference, a photoconductive imaging member comprised of a hole blocking layer, a photogenerating layer, and a charge transport layer, and wherein the hole blocking layer is comprised of a metal oxide; and a mixture of a phenolic compound and a phenolic resin wherein the phenolic compound contains at least two phenolic groups.

Layered photoconductors have been described in numerous U.S. patents, such as U.S. Pat. No. 4,265,990, the disclosure of which is totally incorporated herein by reference, wherein there is illustrated an imaging member comprised of a photogenerating layer, and an aryl amine hole transport layer.

In U.S. Pat. No. 4,587,189, the disclosure of which is totally incorporated herein by reference, there is illustrated a layered imaging member with, for example, a perylene, pigment photogenerating component and an aryl amine component, such as N,N'-diphenyl-N,N'-bis(3-methylphenyl)-1,1'-biphenyl-4,4'-diamine dispersed in a polycarbonate binder as a hole transport layer.

Illustrated in U.S. Pat. No. 5,521,306, the disclosure of which is totally incorporated herein by reference, is a process for the preparation of Type V hydroxygallium phthalocyanine comprising the in situ formation of an alkoxy-bridged gallium phthalocyanine dimer, hydrolyzing the dimer to hydroxygallium phthalocyanine, and subsequently converting the hydroxygallium phthalocyanine product to Type V hydroxygallium phthalocyanine.

Illustrated in U.S. Pat. No. 5,482,811, the disclosure of which is totally incorporated herein by reference, is a process for the preparation of hydroxygallium phthalocyanine photo-

generating pigments which comprises as a first step hydrolyzing a gallium phthalocyanine precursor pigment by dissolving the hydroxygallium phthalocyanine in a strong acid, and then reprecipitating the resulting dissolved pigment in basic aqueous media.

Also, in U.S. Pat. No. 5,473,064, the disclosure of which is totally incorporated herein by reference, there is illustrated a process for the preparation of photogenerating pigments of hydroxygallium phthalocyanine Type V essentially free of chlorine, whereby a pigment precursor Type I chlorogallium phthalocyanine is prepared by reaction of gallium chloride in a solvent, such as N-methylpyrrolidone, present in an amount of from about 10 parts to about 100 parts, and preferably about 19 parts with 1,3-diminoisoindolene (DI<sup>3</sup>) in an amount of from about 1 part to about 10 parts, and preferably about 4 parts of DI<sup>3</sup>, for each part of gallium chloride that is reacted; hydrolyzing said pigment precursor chlorogallium phthalocyanine Type I by standard methods, for example acid pasting, whereby the pigment precursor is dissolved in concentrated sulfuric acid and then reprecipitated in a solvent, such as water, or a dilute ammonia solution, for example from about 10 to about 15 percent; and subsequently treating the resulting hydrolyzed pigment hydroxygallium phthalocyanine Type I with a solvent, such as N,N-dimethylformamide, present in an amount of from about 1 volume part to about 50 volume parts, and more specifically, about 15 volume parts for each weight part of pigment hydroxygallium phthalocyanine that is used by, for example, ball milling the Type I hydroxygallium phthalocyanine pigment in the presence of spherical glass beads, approximately 1 millimeter to 5 millimeters in diameter, at room temperature, about 25° C., for a period of from about 12 hours to about 1 week, and more specifically, about 24 hours.

The appropriate components, such as the supporting substrates, the photogenerating layer components, the charge transport layer components, the overcoating layer components, and the like of the above-recited patents, may be selected for the photoconductors of the present disclosure in embodiments thereof.

#### SUMMARY

The present disclosure in embodiments is directed to multilayered drum, or flexible, belt photoconductors, or devices comprised of a supporting medium like a substrate, a photogenerating layer, and a charge transport layer, including a plurality of charge transport layers, such as a first charge transport layer and a second charge transport layer, and wherein the first charge transport layer in contact with the photogenerating layer contains an additive or dopant, such as a phosphonium salt; and a photoconductor comprised of a supporting medium like a substrate, a photogenerating layer, and a charge transport layer, including a plurality of charge transport layers, such as a first charge transport layer and a second charge transport layer, and wherein at least one of the charge transport layers contains a phosphonium salt additive or dopant; a photoconductor comprised of an optional supporting substrate, a photogenerating layer and at least one charge transport layer containing a phosphonium salt additive or dopant in an amount, for example, of from about 1 to about 1,000 parts per million, and which additive in embodiments is dissolved in the charge transporting layer dispersion solvent, such as methylene chloride, to achieve a number of the advantages illustrated herein.

There is disclosed in embodiments a photoconductor comprising a supporting substrate, a photogenerating layer, and at least one charge transport layer comprised of at least one

charge transport component, and wherein the at least one charge transport layer, such as 1, from about 1 to 4, or 2, contains at least one phosphonium salt; a photoconductor comprised in sequence of an optional supporting substrate, a photogenerating layer, and a charge transport layer; and wherein the charge transport layer contains a phosphonium salt; a photoconductor comprising a supporting substrate, a photogenerating layer, a first hole transport layer and a second hole transport layer, and wherein the first hole transport layer has incorporated therein a phosphonium salt selected from the group consisting of tetradecyl(triethyl)phosphonium chloride, tetradecyl(triethyl)phosphonium decanoate, triethyl(tetradecyl)phosphonium bis 2,4,4-trimethylpentylphosphinate, tetradecyl(triethyl)phosphonium dicyanamide, triisobutyl(methyl)phosphonium tosylate, tetradecyl(triethyl)phosphonium bistriflamide, tetradecyl(triethyl)phosphonium hexafluorophosphate, tetradecyl(triethyl)phosphonium tetrafluoroborate, ethyl tri(butyl)phosphonium diethylphosphate, (N-methyl-N-phenylamino)triethylphosphonium iodide, 2-dimethylaminoethyltrifluorophosphonium bromide, 4-(carboxybutyl)trifluorophosphonium bromide, amyltrifluorophosphonium bromide, tetrabutylphosphonium benzotriazolate, tetrabutylphosphonium tetraphenylborate, tetrakis(hydroxymethyl) phosphonium chloride, tributylmethylphosphonium iodide, and the like, and mixtures thereof, and which salt is present in an amount of from about 2 to about 300 parts per million.

## EMBODIMENTS

Aspects of the present disclosure relate to a photoconductor comprising a supporting substrate, a photogenerating layer, and at least one charge transport layer comprised of at least one charge transport component, and where the photogenerating layer, or charge transport layer contains the additive or dopant as illustrated herein; a photoconductor comprising a supporting substrate, a photogenerating layer, and at least one charge transport layer comprised of at least one charge transport component, and wherein the photogenerating layer contains at least one of an ammonium salt and an imidazolium salt; a photoconductor comprised in sequence of an optional supporting substrate, a photogenerating layer, and a charge transport layer, and wherein the photogenerating layer is comprised of a photogenerating pigment and present in various suitable amounts at least one of tetrabutylammonium fluoride, benzalkonium chloride, (2-methoxyethoxymethyl)triethylammonium chloride, dodecyltrimethylammonium chloride, hexamethonium chloride dihydrate, stachydrine hydrochloride, trimethyl[3-(triethoxysilyl)propyl] ammonium chloride, (ferrocenylmethyl)dodecyldimethyl ammonium bromide, choline bromide, decamethonium bromide, n-octyltrimethylammonium bromide, (ferrocenylmethyl)trimethylammonium iodide, 1,1-dimethyl-4-phenylpiperazinium iodide, tetra-n-hexylammonium iodide, hexadecyltrimethylammonium hydroxide, tris(2-hydroxyethyl)methylammonium hydroxide, benzyltrimethylammonium hydroxide, 1-butyl-1-methyl pyrrolidinium bis(trifluoromethanesulfonyl)imide, bis(tetra-n-butylammonium)tetracyano diphenoxquinodimethane, choline bitartrate, dodecyldimethyl(3-sulfopropyl)ammonium hydroxide inner salt, hexadecyltrimethylammonium hexafluorophosphate, N-fluoro-N'-(chloromethyl)triethylenediamine bis(tetrafluoroborate), n-hexadecyltrimethyl ammonium tetrafluoroborate, tetra-n-butylammonium dichloroaurate, tetra-n-butylammonium difluorotriphenylsilicate, tetra-n-butylammonium difluorotriphenylstannate, and tetra-n-butylammonium tetraphenylborate optionally present in an amount of from about 15 parts per million to about 750 parts per million; a photoconductor wherein the imidazolium salt is at least one of 1,3-di-tertiary-butylimidazolium tetrafluoroborate, N,N'-(isopropyl)imidazolium chloride, imidazolium triflate, N,N'-(adamantyl)imidazolium tetrafluoroborate, 1,3-bis(2,4,6-trimethylphenyl)imidazolium chloride, 1-methyl-3-(3-cyanopropyl)imidazolium dicyanamide, N,N'-bis-(tert-butyl)imidazolium tetrafluoroborate, 1-[bis(4-chlorophenyl)methyl]-3-[2,4-dichloro- $\beta$ -(2,4-dichlorobenzyl)oxy]phenethylimidazolium chloride, 1-butyl-3-(2-pyridinylmethyl)-1H-imidazolium hexafluorophosphate, 4-(3-butyl-1-imidazolino)-1-butanesulfonic acid triflate, 1-methyl-3-(cyanomethyl)imidazolium chloride, 1,3-dimethylimidazolium dimethyl phosphate, 1-butyl-3-methylimidazolium bis(trifluoromethanesulfonyl)imide, 1-butyl-3-methylimidazolium tetrachloroferrate, 1-ethyl-3-methylimidazolium 2-(2-methoxyethoxy)ethyl sulfate, 1-methyl-3-propylimidazolium iodide, and 1,3-di-tertiary-butylimidazolium tetrafluoroborate; a photoconductor wherein the ammonium salt is at least one of tetrabutylammonium fluoride, benzalkonium chloride, (2-methoxyethoxymethyl)triethylammonium chloride, dodecyltrimethylammonium chloride, hexamethonium chloride dihydrate, stachydrine hydrochloride, trimethyl[3-(triethoxysilyl)propyl]ammonium chloride, (ferrocenylmethyl)dodecyltrimethyl ammonium bromide, choline bromide, decamethonium bromide, n-octyltrimethylammonium bromide, (ferrocenylmethyl)trimethylammonium iodide, 1,1-dimethyl-4-phenylpiperazinium iodide, tetra-n-hexylammonium iodide, hexadecyltrimethylammonium hydroxide, tris(2-hydroxyethyl)methylammonium hydroxide, benzyltrimethylammonium hydroxide, 1-butyl-1-methyl pyrrolidinium bis(trifluoromethanesulfonyl)imide, bis(tetra-n-butylammonium)tetracyano diphenoxquinodimethane, choline bitartrate, dodecyldimethyl(3-sulfopropyl)ammonium hydroxide inner salt, hexadecyltrimethylammonium hexafluorophosphate, N-fluoro-N'-(chloromethyl)triethylenediamine bis(tetrafluoroborate), n-hexadecyltrimethyl ammonium tetrafluoroborate, tetra-n-butylammonium dichloroaurate, tetra-n-butylammonium difluorotriphenylsilicate, tetra-n-butylammonium difluorotriphenylstannate, and tetra-n-butylammonium tetraphenylborate optionally present in an amount of from about 15 parts per million to about 750 parts per million; a photoconductor wherein the imidazolium salt is at least one of 1,3-di-tertiary-butylimidazolium tetrafluoroborate, N,N'-(isopropyl)imidazolium chloride, imidazolium triflate, N,N'-(adamantyl)imidazolium tetrafluoroborate, 1,3-bis(2,4,6-trimethylphenyl)imidazolium chloride, 1-methyl-3-(3-cyanopropyl)imidazolium dicyanamide, N,N'-bis-(tert-butyl)imidazolium tetrafluoroborate, 1-[bis(4-chlorophenyl)methyl]-3-[2,4-dichloro- $\beta$ -(2,4-dichlorobenzyl)oxy]phenethylimidazolium chloride, 1-butyl-3-(2-pyridinylmethyl)-1H-imidazolium hexafluorophosphate, 4-(3-butyl-1-imidazolino)-1-butanesulfonic acid triflate, 1-methyl-3-(cyanomethyl)imidazolium chloride, 1,3-dimethylimidazolium dimethyl phosphate, 1-butyl-3-methylimidazolium bis(trifluoromethanesulfonyl)imide, 1-butyl-3-methylimidazolium tetrachloroferrate, 1-ethyl-3-methylimidazolium 2-(2-methoxyethoxy)ethyl sulfate, and 1-methyl-3-propylimidazolium iodide optionally present in an amount of from about 20 parts per million to 1,000 parts per million, and mixtures thereof; a photoconductor wherein the charge transport component is an aryl amine selected from the group consisting of N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine,

tymmonium difluorotriphenylsilicate, tetra-n-butylammonium difluorotriphenylstannate, tetra-n-butylammonium tetraphenylborate, N,N'-(isopropyl)imidazolium chloride, imidazolium triflate, N,N'-(adamantyl)imidazolium tetrafluoroborate, 1,3-bis(2,4,6-trimethylphenyl)imidazolium chloride, 1-methyl-3-(3-cyanopropyl)imidazolium dicyanamide, N,N'-bis-(tert-butyl)imidazolium tetrafluoroborate, 1-[bis(4-chlorophenyl)methyl]-3-[2,4-dichloro- $\beta$ -(2,4-dichlorobenzyl)oxy]phenethylimidazolium chloride, 1-butyl-3-(2-pyridinylmethyl)-1H-imidazolium hexafluorophosphate, 4-(3-butyl-1-imidazolino)-1-butanesulfonic acid triflate, 1-methyl-3-(cyanomethyl)imidazolium chloride, 1,3-dimethylimidazolium dimethyl phosphate, 1-butyl-3-methylimidazolium bis(trifluoromethanesulfonyl)imide, 1-butyl-3-methylimidazolium tetrachloroferrate, 1-ethyl-3-methylimidazolium 2-(2-methoxyethoxy)ethyl sulfate, 1-methyl-3-propylimidazolium iodide, and 1,3-di-tertiary-butylimidazolium tetrafluoroborate; a photoconductor wherein the ammonium salt is at least one of tetrabutylammonium fluoride, benzalkonium chloride, (2-methoxyethoxymethyl)triethylammonium chloride, dodecyltrimethylammonium chloride, hexamethonium chloride dihydrate, stachydrine hydrochloride, trimethyl[3-(triethoxysilyl)propyl]ammonium chloride, (ferrocenylmethyl)dodecyltrimethyl ammonium bromide, choline bromide, decamethonium bromide, n-octyltrimethylammonium bromide, (ferrocenylmethyl)trimethylammonium iodide, 1,1-dimethyl-4-phenylpiperazinium iodide, tetra-n-hexylammonium iodide, hexadecyltrimethylammonium hydroxide, tris(2-hydroxyethyl)methylammonium hydroxide, benzyltrimethylammonium hydroxide, 1-butyl-1-methyl pyrrolidinium bis(trifluoromethanesulfonyl)imide, bis(tetra-n-butylammonium)tetracyano diphenoxquinodimethane, choline bitartrate, dodecyldimethyl(3-sulfopropyl)ammonium hydroxide inner salt, hexadecyltrimethylammonium hexafluorophosphate, N-fluoro-N'-(chloromethyl)triethylenediamine bis(tetrafluoroborate), n-hexadecyltrimethyl ammonium tetrafluoroborate, tetra-n-butylammonium dichloroaurate, tetra-n-butylammonium difluorotriphenylsilicate, tetra-n-butylammonium difluorotriphenylstannate, and tetra-n-butylammonium tetraphenylborate optionally present in an amount of from about 15 parts per million to about 750 parts per million; a photoconductor wherein the imidazolium salt is at least one of 1,3-di-tertiary-butylimidazolium tetrafluoroborate, N,N'-(isopropyl)imidazolium chloride, imidazolium triflate, N,N'-(adamantyl)imidazolium tetrafluoroborate, 1,3-bis(2,4,6-trimethylphenyl)imidazolium chloride, 1-methyl-3-(3-cyanopropyl)imidazolium dicyanamide, N,N'-bis-(tert-butyl)imidazolium tetrafluoroborate, 1-[bis(4-chlorophenyl)methyl]-3-[2,4-dichloro- $\beta$ -(2,4-dichlorobenzyl)oxy]phenethylimidazolium chloride, 1-butyl-3-(2-pyridinylmethyl)-1H-imidazolium hexafluorophosphate, 4-(3-butyl-1-imidazolino)-1-butanesulfonic acid triflate, 1-methyl-3-(cyanomethyl)imidazolium chloride, 1,3-dimethylimidazolium dimethyl phosphate, 1-butyl-3-methylimidazolium bis(trifluoromethanesulfonyl)imide, 1-butyl-3-methylimidazolium tetrachloroferrate, 1-ethyl-3-methylimidazolium 2-(2-methoxyethoxy)ethyl sulfate, and 1-methyl-3-propylimidazolium iodide optionally present in an amount of from about 20 parts per million to 1,000 parts per million, and mixtures thereof; a photoconductor wherein the charge transport component is an aryl amine selected from the group consisting of N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine,

N,N'-bis(4-butylphenyl)-N,N'-bis-(4-isopropylphenyl)-[p-terphenyl]-4,4"-diamine, N,N'-bis(4-butylphenyl)-N,N'-bis-(2-ethyl-6-methylphenyl)-[p-terphenyl]-4,4"-diamine, N,N'-bis(4-butylphenyl)-N,N'-bis-(2,5-dimethylphenyl)-[p-terphenyl]-4,4"-diamine, N,N'-diphenyl-N,N'-bis(3-chlorophenyl)-[p-terphenyl]-4,4"-diamine, and mixtures thereof; and wherein the at least one charge transport layer is from 1 to about 4, and wherein the salt is tetrabutylammonium fluoride, benzalkonium chloride, (2-methoxyethoxymethyl) triethylammonium chloride, dodecyltrimethylammonium chloride, hexamethonium chloride dihydrate, stachydrine hydrochloride, trimethyl[3-(triethoxysilyl)propyl]ammonium chloride, (ferrocenylmethyl)dodecyl dimethylammonium bromide, choline bromide, decamethonium bromide, n-octyltrimethylammonium bromide, (ferrocenylmethyl)trimethylammonium iodide, 1,1-dimethyl-4-phenylpiperazinium iodide, tetra-n-hexylammonium iodide, hexadecyltrimethylammonium hydroxide, tris(2-hydroxyethyl) methylammonium hydroxide, benzyltrimethylammonium hydroxide, 1-butyl-1-methyl pyrrolidinium bis(trifluoromethanesulfonyl)imide, bis(tetra-n-butylammonium)tetra-cyano diphenoquinodimide, choline bitartrate, dodecyltrimethyl(3-sulfopropyl) ammonium hydroxide inner salt, hexadecyltrimethylammonium hexafluorophosphate, N-fluoro-N'-(chloromethyl)triethylenediamine bis(tetrafluoroborate), n-hexadecyltrimethylammonium tetrafluoroborate, tetra-n-butylammonium dichloroaurate, tetra-n-butylammonium difluorotriphenylsilicate, tetra-n-butylammonium difluorotriphenylstannate, tetra-n-butylammonium tetraphenylborate, 10 N,N'-(isopropyl)imidazolium chloride, imidazolium triflate, N,N'-(adamantyl)imidazolium tetrafluoroborate, 1,3-bis(2,4,6-trimethylphenyl)imidazolium chloride, 1-methyl-3-(3-cyanopropyl) imidazolium dicyanamide, N,N'-bis-(tert-butyl)imidazolium tetrafluoroborate, 1-[bis(4-chlorophenyl)methyl]-3-[2,4-dichloro- $\beta$ -(2,4-dichlorobenzoyloxy)phenethyl]imidazolium chloride, 1-butyl-3-(2-pyridinylmethyl)-1H-imidazolium hexafluorophosphate, 20 4-(3-butyl-1-imidazolio)-1-butanesulfonic acid triflate, 1-methyl-3-(cyanomethyl)imidazolium chloride, 1,3-dimethylimidazolium dimethyl phosphate, 1-butyl-3-methylimidazolium bis(trifluoromethanesulfonyl)imide, 1-butyl-3-methylimidazolium tetrachloroferrate, 1-ethyl-3-methylimidazolium 2-(2-methoxyethoxy)ethyl sulfate, 25 1-methyl-3-propylimidazolium iodide, or 1,3-di-tertiary-butylimidazolium tetrafluoroborate; and which additive is present in an amount of from about 20 to about 800 parts per million; a flexible photoconductive imaging member comprised in sequence of a supporting substrate, an additive containing photogenerating layer thereover, a charge transport layer, and a protective top overcoating layer; a photoconductor which includes a hole blocking layer and an adhesive layer where the adhesive layer is situated between the hole blocking layer and the photogenerating layer, and the hole blocking layer is situated between the substrate and the adhesive layer; and a photoconductor wherein the additive or dopant can be selected in various effective amounts, such as for example, in parts per million, like from about 1 to about 1,000, and from 30 about 10 to about 500 parts per million of the additive.

bis(tetra-n-butylammonium) tetracyanodiphenoquinodimethanide, choline bitartrate, dodecyltrimethyl(3-sulfopropyl)ammonium hydroxide inner salt, hexadecyltrimethylammonium hexafluorophosphate, N-fluoro-N'-(chloromethyl) triethylenediamine bis(tetrafluoroborate), n-hexadecyltrimethylammonium tetrafluoroborate, tetra-n-butylammonium dichloroaurate, tetra-n-butylammonium difluorotriphenylsilicate, tetra-n-butylammonium difluorotriphenylstannate, tetra-n-butylammonium tetraphenylborate, 10 N,N'-(isopropyl)imidazolium chloride, imidazolium triflate, N,N'-(adamantyl)imidazolium tetrafluoroborate, 1,3-bis(2,4,6-trimethylphenyl)imidazolium chloride, 1-methyl-3-(3-cyanopropyl) imidazolium dicyanamide, N,N'-bis-(tert-butyl)imidazolium tetrafluoroborate, 1-[bis(4-chlorophenyl)methyl]-3-[2,4-dichloro- $\beta$ -(2,4-dichlorobenzoyloxy)phenethyl]imidazolium chloride, 1-butyl-3-(2-pyridinylmethyl)-1H-imidazolium hexafluorophosphate, 20 4-(3-butyl-1-imidazolio)-1-butanesulfonic acid triflate, 1-methyl-3-(cyanomethyl)imidazolium chloride, 1,3-dimethylimidazolium dimethyl phosphate, 1-butyl-3-methylimidazolium bis(trifluoromethanesulfonyl)imide, 1-butyl-3-methylimidazolium tetrachloroferrate, 1-ethyl-3-methylimidazolium 2-(2-methoxyethoxy)ethyl sulfate, 25 1-methyl-3-propylimidazolium iodide, or 1,3-di-tertiary-butylimidazolium tetrafluoroborate; and which additive is present in an amount of from about 20 to about 800 parts per million; a flexible photoconductive imaging member comprised in sequence of a supporting substrate, an additive containing photogenerating layer thereover, a charge transport layer, and a protective top overcoating layer; a photoconductor which includes a hole blocking layer and an adhesive layer where the adhesive layer is situated between the hole blocking layer and the photogenerating layer, and the hole blocking layer is situated between the substrate and the adhesive layer; and a photoconductor wherein the additive or dopant can be selected in various effective amounts, such as for example, in parts per million, like from about 1 to about 1,000, and from 30 about 10 to about 500 parts per million of the additive.

## ADDITIVE/DOPANT EXAMPLES

Examples of the additive or dopant which can function as a charge blocking agent present, for example, in various amounts in parts per million of from about 1 to about 1,000, from about 10 to about 500, from about 20 to about 200, from about 0.00 to about 10 weight percent include, for example, a number of known suitable components, such as phosphonium salts, ammonium salts, and imidazolium salts.

Specific examples of phosphonium salts, which in embodiments have been referred to as ionic liquids, contained in at least one charge transport layer, and more specifically, in a first charge transport layer in contact with the photogenerating layer, and which first charge transport layer is situated between a second charge transport layer and the photogenerating layer, are tetradecyl(triethyl)phosphonium chloride, tetradecyl(triethyl)phosphonium decanoate, triisobutyl(methyl)phosphonium tosylate, trihexyl(tetradecyl)phosphonium bis 2,4,4-trimethylpentylphosphinate, tetradecyl(triethyl)phosphonium dicyanamide, tetradecyl(triethyl)phosphonium bistriflamide, tetradecyl(triethyl)phosphonium hexafluorophosphate, tetradecyl(triethyl)phosphonium tetrafluoroborate, ethyl tri(butyl)phosphonium diethylphosphate, and the like, and mixtures thereof. In embodiments, the phosphonium salts selected can be represented, for example, by the following formulas/structures



11

In embodiments, examples of phosphonium salts contained in at least one charge transport layer, and more specifically, in a first charge transport layer in contact with the photogenerating layer, and which first charge transport layer is situated between a second charge transport layer and the photogenerating layer are (N-methyl-N-phenylamino)triphenylphosphonium iodide, 2-dimethylaminoethyl triphenylphosphonium bromide, 4-(carboxybutyl)triphenylphosphonium bromide, amyltriphenylphosphonium bromide, tetrabutylphosphonium benzotriazolate, tetrabutylphosphonium tetraphenylborate, tetrakis(hydroxymethyl)phosphonium chloride, tributylmethylphosphonium iodide, and the like, and mixtures thereof, may be represented by the following formulas/structures



12

-continued



These and other similar salts, including for example, alkyl salts, halosalts, derivative salts, and the like, can be present in the charge transport layer in various suitable amounts, such as from about 5 to about 5,000, from about 10 to about 3,000, from about 10 to about 500, from about 20 to about 300, from about 40 to about 150, from about 500 to about 1,500 parts per million, or in embodiments from about 0.001 to about 3 weight percent based on the charge transport layer components of the charge transport component, the resin binder, optional known additives, and the phosphonium salt, and wherein the salt can be present in or incorporated into each charge transport layer, less than each charge transport layer, in one charge transport layer, and the like.

Quaternary ammonium cation examples include positively charged polyatomic ions of the formula  $NR_4^+$  with R being alkyl group, which alkyl can be the same or dissimilar, and which alkyl groups can be connected. Unlike the ammonium ion  $NH_4^+$  itself and a number of primary, secondary, or tertiary ammonium cations, the quaternary ammonium cations are permanently charged, independent of the pH of the solution thereof. Quaternary ammonium salts or quaternary ammonium compounds that can be selected as a dopant can be referred to as salts of quaternary ammonium cations with an anion.

Typical ammonium salts include ammonium fluorides, ammonium chlorides, ammonium bromides, ammonium iodides, ammonium hydroxides, and ammonium salts with other anions.

Examples of ammonium fluorides include tetrabutylammonium fluoride represented as follows, and the like



Examples of ammonium chlorides include benzalkonium chloride, (2-methoxyethoxymethyl)triethylammonium chloride, dodecyltrimethylammonium chloride, hexamethonium chloride dihydrate, stachydrine hydrochloride, trimethyl[3-(triethoxysilyl)propyl]ammonium chloride, represented as follows, and the like



Examples of ammonium bromides include (ferrocenylmethyl) dodecyldimethylammonium bromide, choline bromide, decamethonium bromide, n-octyltrimethylammonium bromide, represented as follows, and the like



Examples of ammonium iodides include (ferrocenylmethyl) trimethylammonium iodide, 1,1-dimethyl-4-phenylpiperazinium iodide, tetra-n-hexylammonium iodide, represented as follows, and the like



Examples of ammonium hydroxides include hexadecyltrimethylammonium hydroxide, tris(2-hydroxyethyl)methyl-

lammonium hydroxide, benzyltrimethylammonium hydroxide, represented as follows, and the like



15 Examples of ammonium salts are 1-butyl-1-methylpyrro-  
lidinium bis(trifluoromethanesulfonyl)imide, bis(tetra-n-bu-  
tylammonium) tetracyanodiphenoquinodimethanide, cho-  
line bitartrate, dodecyltrimethyl(3-sulfopropyl)ammonium  
20 hydroxide inner salt, hexadecyltrimethylammonium  
hexafluorophosphate, N-fluoro-N'-chloromethyl)triethyl-  
enediamine bis(tetrafluoroborate), n-hexadecyltrimethylam-  
monium tetrafluoroborate, tetra-n-butylammonium dichloro-  
25 aurate, tetra-n-butylammonium difluorotriphenylsilicate,  
tetra-n-butylammonium difluorotriphenylstannate, tetra-n-  
butylammonium tetraphenylborate, represented as follows,  
and the like



15

-continued



2

143

4

4

5

16

-continued



6

6



Imidazolium salt examples that can be selected as the dopant include 1,3-di-tertiary-butylimidazolium tetrafluoroborate, N,N'-(isopropyl)imidazolium chloride, imidazolium triflate, N,N'-(adamantyl)imidazolium tetrafluoroborate, 1,3-bis(2,4,6-trimethylphenyl)imidazolium chloride, 1-methyl-3-(3-cyanopropyl)imidazolium dicyanamide, 1-[bis(4-chlorophenyl)methyl]-3-[2,4-dichloro- $\beta$ -(2,4-dichlorobenzyl)oxy]phenethylimidazolium chloride, 1-butyl-3-(2-pyridinylmethyl)-1H-imidazolium hexafluorophosphate, 4-(3-butyl-1-imidazolio)-1-butanesulfonic acid triflate, 1-methyl-3-(cyanomethyl)imidazolium chloride, 1,3-dimethylimidazolium dimethyl phosphate, 1-butyl-3-methylimidazolium bis(trifluoromethanesulfonyl)imide, 1-butyl-3-methylimidazolium tetrachloroferrate, 1-ethyl-3-methylimidazolium 2-(2-methoxyethoxy)ethyl sulfate, 1-methyl-3-propylimidazolium iodide, represented as follows, and the like



Photoconductor Layer Components

The thickness of the photoconductor substrate layer may depend on various factors, including economical considerations, desired electrical characteristics, adequate flexibility, and the like, thus this layer may be of substantial thickness, for example over 3,000 microns, such as from about 1,000 to about 2,000 microns, from about 500 to about 1,000 microns, or from about 300 to about 700 microns ("about" throughout includes all values in between the values recited), or of a minimum thickness. In embodiments, the thickness of this layer is from about 75 microns to about 300 microns, or from about 100 to about 150 microns. In embodiments, the photoconductor can be free of a substrate, for example the layer usually in contact with the substrate can be increased in thickness. For a photoconductor drum, the substrate or supporting medium may be of a substantial thickness of, for example, up to many centimeters or of a minimum thickness of less than a millimeter. Similarly, a flexible belt may be of a substantial thickness of, for example, about 250 micrometers, or of a minimum thickness of less than about 50 micrometers, provided there are no adverse effects on the final electrophotographic device.

Also, the photoconductor may in embodiments include a blocking layer, an adhesive layer, a top overcoating protective layer, and an anticurl backing layer.

The photoconductor substrate may be opaque, substantially opaque, or substantially transparent, and may comprise any suitable material that, for example, permits the photoconductor layers to be supported. Accordingly, the substrate may comprise a number of known layers, and more specifically, the substrate can be comprised of an electrically nonconduc-

tive or conductive material such as an inorganic or an organic composition. As electrically nonconducting materials, there may be selected various resins known for this purpose including polyesters, polycarbonates, polyamides, polyurethanes, and the like, which are flexible as thin webs. An electrically conducting substrate may comprise any suitable metal of, for example, aluminum, nickel, steel, copper, and the like, or a polymeric material filled with an electrically conducting substance, such as carbon, metallic powder, and the like, or an organic electrically conducting material. The electrically insulating or conductive substrate may be in the form of an endless flexible belt, a web, a rigid cylinder, a sheet, and the like.

In embodiments where the substrate layer is to be rendered conductive, the surface thereof may be rendered electrically conductive by an electrically conductive coating. The conductive coating may vary in thickness depending upon the optical transparency, degree of flexibility desired, and economic factors, and in embodiments this layer can be of a thickness of from about 0.05 micron to about 5 microns.

Illustrative examples of substrates are as illustrated herein, and more specifically, supporting substrate layers selected for the photoconductors of the present disclosure comprise a layer of insulating material including inorganic or organic polymeric materials, such as MYLAR® a commercially available polymer, MYLAR® containing titanium, a layer of an organic or inorganic material having a semiconductive surface layer, such as indium tin oxide, or aluminum arranged thereon, or a conductive material inclusive of aluminum, chromium, nickel, brass, or the like. The substrate may be flexible, seamless, or rigid, and may have a number of many different configurations, such as for example, a plate, a cylindrical drum, a scroll, an endless flexible belt, and the like. In embodiments, the substrate is in the form of a seamless flexible belt. In some situations, it may be desirable to coat on the back of the substrate, particularly when the substrate is a flexible organic polymeric material, an anticurl layer, such as for example polycarbonate materials commercially available as MAKROLON®.

Generally, the photogenerating layer can contain known photogenerating pigments, such as metal phthalocyanines, metal free phthalocyanines, and more specifically alkylhydroxyl gallium phthalocyanines, hydroxyl gallium phthalocyanines, chlorogallium phthalocyanines, perylenes, especially bis(benzimidazo)perylene, titanyl phthalocyanines, and the like, and yet more specifically, vanadyl phthalocyanines, Type V hydroxyl gallium phthalocyanines, and inorganic components such as selenium, selenium alloys, and trigonal selenium. The photogenerating pigment can be dispersed in a resin binder similar to the resin binders selected for the charge transport layer, or alternatively no resin binder need be present. Generally, the thickness of the photogenerating layer depends on a number of factors, including the thicknesses of the other layers and the amount of photogenerating material contained in the photogenerating layer. Accordingly, this layer can be of a thickness of, for example, from about 0.05 micron to about 10 microns, and more specifically, from about 0.25 micron to about 2 microns when, for example, the photogenerating compositions are present in an amount of from about 30 to about 75 percent by volume.

In embodiments, the photogenerating component or pigment is present in a resinous binder in various amounts, inclusive of 100 percent by weight based on the weight of the photogenerating components that are present. Generally, however, from about 5 percent by volume to about 95 percent by volume of the photogenerating pigment is dispersed in about 95 percent by volume to about 5 percent by volume of

the resinous binder, or from about 20 percent by volume to about 30 percent by volume of the photogenerating pigment is dispersed in about 70 percent by volume to about 80 percent by volume of the resinous binder composition. In one embodiment, about 90 percent by volume of the photogenerating pigment is dispersed in about 10 percent by volume of the resinous binder composition, and which resin may be selected from a number of known polymers, such as poly(vinyl butyral), poly(vinyl carbazole), polyesters, polycarbonates, poly(vinyl chloride), polyacrylates and methacrylates, copolymers of vinyl chloride and vinyl acetate, phenolic resins, polyurethanes, poly(vinyl alcohol), polyacrylonitrile, polystyrene, and the like. It is desirable to select a coating solvent that does not substantially disturb or adversely affect the other previously coated layers of the device. Examples of coating solvents for the photogenerating layer are ketones, alcohols, aromatic hydrocarbons, halogenated aliphatic hydrocarbons, ethers, amines, amides, esters, and the like. Specific solvent examples are cyclohexanone, acetone, methyl ethyl ketone, methanol, ethanol, butanol, amyl alcohol, toluene, xylene, chlorobenzene, carbon tetrachloride, chloroform, methylene chloride, trichloroethylene, tetrahydrofuran, dioxane, diethyl ether, dimethyl formamide, dimethyl acetamide, butyl acetate, ethyl acetate, methoxyethyl acetate, and the like.

In embodiments, examples of polymeric binder materials that can be selected as the matrix for the photogenerating layer components are known and include thermoplastic and thermosetting resins, such as polycarbonates, polyesters, polyamides, polyurethanes, polystyrenes, polyarylethers, polyarylsulfones, polybutadienes, polysulfones, polyethersulfones, polyethylenes, polypropylenes, polyimides, polymethylpentenes, poly(phenylene sulfides), poly(vinyl acetate), polysiloxanes, polyacrylates, polyvinyl acetals, polyamides, polyimides, amino resins, phenylene oxide resins, terephthalic acid resins, phenoxy resins, epoxy resins, phenolic resins, polystyrene, and acrylonitrile copolymers, poly(vinyl chloride), vinyl chloride and vinyl acetate copolymers, acrylate copolymers, alkyl resins, cellulosic film formers, poly(amideimide), styrenebutadiene copolymers, vinylidene chloride-vinyl chloride copolymers, vinyl acetate-vinylidene chloride copolymers, styrene-alkyd resins, poly(vinyl carbazole), and the like. These polymers may be block, random, or alternating copolymers.

Various suitable and conventional known processes may be used to mix, and thereafter apply the photogenerating layer coating mixture like spraying, dip coating, roll coating, wire wound rod coating, vacuum sublimation, and the like. For some applications, the photogenerating layer may be fabricated in a dot or line pattern. Removal of the solvent of a solvent-coated layer may be effected by any known conventional techniques such as oven drying, infrared radiation drying, air drying, and the like.

The dopant in embodiments can be added to the photogenerating dispersion or to the charge transport mixture, and such dopant is, more specifically, substantially dissolved in the photogenerating dispersion solvent or in the charge transport layer mixture. Moreover, the dopant or additive can be included in both the photogenerating layer, and in the charge transport layer or layers.

The final dry thickness of the photogenerating layer is as illustrated herein, and can be, for example, from about 0.01 to about 30 microns after being dried at, for example, about 40° C. to about 150° C. for about 15 to about 90 minutes. More specifically, a photogenerating layer of a thickness, for example, of from about 0.1 to about 30, or from about 0.5 to about 2 microns can be applied to or deposited on the sub-

strate, on other surfaces in between the substrate and the charge transport layer, and the like. A charge blocking layer or hole blocking layer may optionally be applied to the electrically conductive surface prior to the application of a photogenerating layer. When desired, an adhesive layer may be included between the charge blocking or hole blocking layer or interfacial layer and the photogenerating layer. Usually, the photogenerating layer is applied onto the blocking layer and a charge transport layer or plurality of charge transport layers are formed on the photogenerating layer. This structure may have the photogenerating layer on top of or below the charge transport layer.

In embodiments, a suitable known adhesive layer can be included in the photoconductor. Typical adhesive layer materials include, for example, polyesters, polyurethanes, and the like. The adhesive layer thickness can vary and in embodiments is, for example, from about 0.05 micrometer (500 Angstroms) to about 0.3 micrometer (3,000 Angstroms). The adhesive layer can be deposited on the hole blocking layer by spraying, dip coating, roll coating, wire wound rod coating, gravure coating, Bird applicator coating, and the like. Drying of the deposited coating may be effected by, for example, oven drying, infrared radiation drying, air drying, and the like.

As an optional adhesive layer or layers usually in contact with or situated between the hole blocking layer and the photogenerating layer, there can be selected various known substances inclusive of copolymers, polyamides, poly(vinyl butyral), poly(vinyl alcohol), polyurethane, and polyacrylonitrile. This layer is, for example, of a thickness of from about 0.001 micron to about 1 micron, or from about 0.1 to about 0.5 micron. Optionally, this layer may contain effective suitable amounts, for example from about 1 to about 10 weight percent, of conductive and nonconductive particles, such as zinc oxide, titanium dioxide, silicon nitride, carbon black, and the like, to provide, for example, in embodiments of the present disclosure further desirable electrical and optical properties.

The hole blocking or undercoat layer for the imaging members of the present disclosure can contain a number of components including known hole blocking components, such as amino silanes, doped metal oxides, a metal oxide like titanium, chromium, zinc, tin and the like; a mixture of phenolic compounds and a phenolic resin, or a mixture of two phenolic resins, and optionally a dopant such as  $\text{SiO}_2$ . The phenolic compounds usually contain at least two phenol groups, such as bisphenol A (4,4'-isopropylidenediphenol), E (4,4'-ethylenebisphenol), F (bis(4-hydroxyphenyl)methane), M (4,4'-(1,3-phenylene)bisphenol), P (4,4'-(1,4-phenylene)bisphenol), S (4,4'-sulfonyldiphenol), and Z (4,4'-cyclohexylidenebisphenol); hexafluorobisphenol A (4,4'-(hexafluoro isopropylidene) diphenol), resorcinol, hydroxyquinone, catechin, and the like.

The hole blocking layer can be, for example, comprised of from about 20 weight percent to about 80 weight percent, and more specifically, from about 55 weight percent to about 65 weight percent of a suitable component like a metal oxide, such as  $\text{TiO}_2$ , from about 20 weight percent to about 70 weight percent, and more specifically, from about 25 weight percent to about 50 weight percent of a phenolic resin; from about 2 weight percent to about 20 weight percent, and more specifically, from about 5 weight percent to about 15 weight percent of a phenolic compound preferably containing at least two phenol groups, such as bisphenol S, and from about 2 weight percent to about 15 weight percent, and more specifically, from about 4 weight percent to about 10 weight percent of a plywood suppression dopant, such as  $\text{SiO}_2$ . The hole

21

blocking layer coating dispersion can, for example, be prepared as follows. The metal oxide/phenolic resin dispersion is first prepared by ball milling or dynomilling until the median particle size of the metal oxide in the dispersion is less than about 10 nanometers, for example from about 5 to about 9. To the above dispersion are added a phenolic compound and dopant followed by mixing. The hole blocking layer coating dispersion can be applied by dip coating or web coating, and the layer can be thermally cured after coating. The hole blocking layer resulting is, for example, of a thickness of from about 0.01 micron to about 30 microns, and more specifically, from about 0.1 micron to about 8 microns. Examples of phenolic resins include formaldehyde polymers with phenol, p-tert-butylphenol, cresol, such as VARCUM™ 29159 and 29101 (available from OxyChem Company), and DURITE™ 97 (available from Borden Chemical); formaldehyde polymers with ammonia, cresol and phenol, such as VARCUM™ 29112 (available from OxyChem Company); formaldehyde polymers with 4,4'-(1-methylethylidene)bisphenol, such as VARCUM™ 29108 and 29116 (available from OxyChem Company); formaldehyde polymers with cresol and phenol, such as VARCUM™ 29457 (available from OxyChem Company), DURITE™ SD-423A, SD-422A (available from Borden Chemical); or formaldehyde polymers with phenol and p-tert-butylphenol, such as DURITE™ ESD 556C (available from Borden Chemical).

The optional hole blocking layer may be applied to the substrate. Any suitable and conventional blocking layer capable of forming an electronic barrier to holes between the adjacent photoconductive layer (or electrophotographic imaging layer) and the underlying conductive surface of substrate may be selected.

A number of charge transport compounds can be included in the charge transport layer, which layer generally is of a thickness of from about 5 microns to about 80 microns, and more specifically, of a thickness of from about 10 microns to about 40 microns. Examples of charge transport components are aryl amines of the following formulas/structures



wherein X is a suitable hydrocarbon like alkyl, alkoxy, aryl, and derivatives thereof; a halogen, or mixtures thereof, and especially those substituents selected from the group consisting of Cl and CH<sub>3</sub>; and molecules of the following formulas

22



wherein X, Y and Z are independently alkyl, alkoxy, aryl, a halogen, or mixtures thereof, and wherein at least one of Y and Z are present.

Alkyl and alkoxy contain, for example, from 1 to about 25 carbon atoms, and more specifically, from 1 to about 12 carbon atoms, such as methyl, ethyl, propyl, butyl, pentyl, and the corresponding alkoxides. Aryl can contain from 6 to about 36 carbon atoms, such as phenyl, and the like. Halogen includes chloride, bromide, iodide and fluoride. Substituted alkyls, alkoxy, and aryls can also be selected in embodiments.

Examples of specific aryl amines that can be selected for the charge transport layer include N,N'-diphenyl-N,N'-bis(alkylphenyl)-1,1-biphenyl-4,4'-diamine wherein alkyl is selected from the group consisting of methyl, ethyl, propyl, butyl, hexyl, and the like; N,N'-diphenyl-N,N'-bis(halophenyl)-1,1-biphenyl-4,4'-diamine wherein the halo substituent is a chloro substituent; N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis-(4-isopropylphenyl)-[p-terphenyl]-4,4"-diamine, N,N'-bis(4-butylphenyl)-N,N'-bis(2-ethyl-6-methylphenyl)-[p-terphenyl]-4,4"-diamine, N,N'-bis(4-butylphenyl)-N,N'-bis-(2,5-dimethylphenyl)-[p-terphenyl]-4,4"-diamine, N,N'-diphenyl-N,N'-bis(3-chlorophenyl)-[p-terphenyl]-4,4"-diamine, and the like. Other known charge transport layer molecules can be selected, reference for example, U.S. Pat. Nos. 4,921,773 and 4,464,450, the disclosures of which are totally incorporated herein by reference.

Examples of the binder materials selected for the charge transport layers include polycarbonates, polyarylates, acrylate polymers, vinyl polymers, cellulose polymers, polyesters, polysiloxanes, polyamides, polyurethanes, poly(cycloolefins), epoxies, and random or alternating copolymers thereof; and more specifically, polycarbonates such as poly(4,4'-isopropylidene-diphenylene) carbonate (also referred to as bisphenol-A-polycarbonate), poly(4,4'-cyclohexylidene-diphenylene) carbonate (also referred to as bisphenol-Z-polycarbonate), poly(4,4'-isopropylidene-3,3'-dimethyl-diphenyl) carbonate (also referred to as bisphenol-C-polycarbonate), and the like. In embodiments, electrically inactive binders are comprised of polycarbonate resins with a molecular weight of from about 20,000 to about 100,000, or with a molecular weight M<sub>w</sub> of from about 50,000 to about 100,000. Generally, the transport layer contains from about

10 to about 75 percent by weight of the charge transport material, and more specifically, from about 35 percent to about 50 percent of this material.

The charge transport layer or layers, and more specifically, a first charge transport in contact with the photogenerating layer, and thereover a top or second charge transport overcoating layer may comprise charge transporting small molecules dissolved or molecularly dispersed in a film forming electrically inert polymer such as a polycarbonate. In embodiments, "dissolved" refers, for example, to forming a solution in which the small molecule is dissolved in the polymer to form a homogeneous phase; and "molecularly dispersed in embodiments" refers, for example, to charge transporting molecules dispersed in the polymer, the small molecules being dispersed in the polymer on a molecular scale. Various charge transporting or electrically active small molecules may be selected for the charge transport layer or layers. In embodiments, charge transport refers, for example, to charge transporting molecules as a monomer that allows the free charge generated in the photogenerating layer to be transported across the transport layer.

Examples of hole transporting molecules present, for example, in an amount of from about 50 to about 75 weight percent include, for example, pyrazolines such as 1-phenyl-3-(4'-diethylamino styryl)-5-(4"-diethylamino phenyl)pyrazoline; aryl amines such as N,N'-diphenyl-N,N'-bis(3-methylphenyl)-(1,1'-biphenyl)-4,4'-diamine, N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis(4-isopropylphenyl)-[p-terphenyl]-4,4"-diamine, N,N'-bis(4-butylphenyl)-N,N'-bis(2-ethyl-6-methylphenyl)-[p-terphenyl]-4,4"-diamine, N,N'-bis(4-butylphenyl)-N,N'-bis(2,5-dimethylphenyl)-[p-terphenyl]-4,4"-diamine, N,N'-diphenyl-N,N'-bis(3-chlorophenyl)-[p-terphenyl]-4,4"-diamine; hydrazones such as N-phenyl-N-methyl-3-(9-ethyl carbazyl hydrazone and 4-diethyl amino benzaldehyde-1,2-diphenyl hydrazone; and oxadiazoles such as 2,5-bis(4-N,N'-diethylaminophenyl)-1,2,4-oxadiazole, stilbenes, and the like. However, in embodiments to minimize or avoid cycle-up in equipment, such as printers, with high throughput, the charge transport layer should be substantially free (less than about two percent) of di or triamino-triphenyl methane. A small molecule charge transporting compound that permits injection of holes into the photogenerating layer with high efficiency and transports them across the charge transport layer with short transit times includes N,N'-diphenyl-N,N'-bis(3-methylphenyl)-(1,1'-biphenyl)-4,4'-diamine, N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis(4-isopropylphenyl)-[p-terphenyl]-4,4"-diamine, N,N'-bis(4-butylphenyl)-N,N'-bis(2-ethyl-6-methylphenyl)-[p-terphenyl]-4,4"-diamine, N,N'-bis(4-butylphenyl)-N,N'-bis(2,5-dimethylphenyl)-[p-terphenyl]-4,4"-diamine, and N,N'-diphenyl-N,N'-bis(3-chlorophenyl)-[p-terphenyl]-4,4"-diamine, or mixtures thereof. If desired, the charge transport material in the charge transport layer may comprise a polymeric charge transport material or a combination of a small molecule charge transport material and a polymeric charge transport material.

Examples of components or materials optionally incorporated into the charge transport layers or at least one charge transport layer to, for example, enable excellent lateral charge migration (LCM) resistance include hindered phenolic anti-

oxidants, such as tetrakis methylene(3,5-di-tert-butyl-4-hydroxy hydrocinnamate) methane (IRGANOX<sup>TM</sup> 1010, available from Ciba Specialty Chemical), butylated hydroxytoluene (BHT), and other hindered phenolic antioxidants including SUMILIZER<sup>TM</sup> BHT-R, MDP-S, BBM-S, WX-R, NW, BP-76, BP-101, GA-80, GM and GS (available from Sumitomo Chemical Co., Ltd.), IRGANOX<sup>TM</sup> 1035, 1076, 1098, 1135, 1141, 1222, 1330, 1425WL, 1520L, 245, 259, 3114, 3790, 5057 and 565 (available from Ciba Specialties Chemicals), and ADEKA STAB<sup>TM</sup> AO-20, AO-30, AO-40, AO-50, AO-60, AO-70, AO-80 and AO-330 (available from Asahi Denka Co., Ltd.); hindered amine antioxidants such as SANOLTM LS-2626, LS-765, LS-770 and LS-744 (available from SNKYO CO., Ltd.), TINUWIN<sup>TM</sup> 144 and 622LD (available from Ciba Specialties Chemicals), MARK<sup>TM</sup> LA57, LA67, LA62, LA68 and LA63 (available from Asahi Denka Co., Ltd.), and SUMILIZER<sup>TM</sup> TPS (available from Sumitomo Chemical Co., Ltd.); thioether antioxidants such as SUMILIZER<sup>TM</sup> TP-D (available from Sumitomo Chemical Co., Ltd.); phosphite antioxidants such as MARK<sup>TM</sup> 2112, PEP-8, PEP-24G, PEP-36, 329K and HP-10 (available from Asahi Denka Co., Ltd.); other molecules such as bis(4-diethylamino-2-methylphenyl) phenylmethane (BDETPM), bis-[2-methyl-4-(N-2-hydroxyethyl-N-ethylaminophenyl)]-phenylmethane (DHTPM), and the like. The weight percent of the antioxidant in at least one of the charge transport layers is from about 0 to about 20, from about 1 to about 10, or from about 3 to about 8 weight percent.

A number of processes may be used to mix, and thereafter apply the charge transport layer or layers coating mixture to the photogenerating layer. Typical application techniques include spraying, dip coating, roll coating, wire wound rod coating, and the like. Drying of the charge transport deposited coating may be effected by any suitable conventional technique such as oven drying, infrared radiation drying, air drying, and the like.

The thickness of each of the charge transport layers in embodiments is from about 10 to about 70 micrometers or microns, but thicknesses outside this range may in embodiments also be selected. The charge transport layer should be an insulator to the extent that an electrostatic charge placed on the hole transport layer is not conducted in the absence of illumination at a rate sufficient to prevent formation and retention of an electrostatic latent image thereon. In general, the ratio of the thickness of the charge transport layer to the photogenerating layer can be from about 2:1 to 200:1, and in some instances 400:1. The charge transport layer is substantially nonabsorbing to visible light or radiation in the region of intended use, but is electrically "active" in that it allows the injection of photogenerated holes from the photoconductive layer, or photogenerating layer, and allows these holes to be transported through itself to selectively discharge a surface charge on the surface of the active layer. Typical application techniques include spraying, dip coating, roll coating, wire wound rod coating, and the like. Drying of the deposited coating may be effected by any suitable conventional technique, such as oven drying, infrared radiation drying, air drying, and the like. An optional overcoating may be applied over the charge transport layer to provide abrasion protection.

The present disclosure in embodiments thereof relate to a photoconductive imaging member comprised of a supporting substrate, an additive containing photogenerating layer, a charge blocking containing charge transport layer, and an overcoating charge transport layer; a photoconductive member with a photogenerating layer of a thickness of from about 0.1 to about 10 microns, and at least one transport layer each of a thickness of from about 5 to about 100 microns; a mem-

ber wherein the thickness of the photogenerating layer is from about 0.1 to about 4 microns; a member wherein the photogenerating layer contains a polymer binder; a member wherein the binder is present in an amount of from about 50 to about 90 percent by weight, and wherein the total of all layer components is about 100 percent; a member wherein the photogenerating component is a hydroxygallium phthalocyanine that absorbs light of a wavelength of from about 370 to about 950 nanometers; an imaging member wherein the supporting substrate is comprised of a conductive substrate comprised of a metal; an imaging member wherein the conductive substrate is aluminum, aluminized polyethylene terephthalate, or titanized polyethylene terephthalate; a photoconductor wherein the photogenerating resinous binder is selected from the group consisting of polyesters, polyvinyl butyral, polycarbonates, polystyrene-*b*-polyvinyl pyridine, and polyvinyl formals; an imaging member wherein the photogenerating pigment is a metal free phthalocyanine; a photoconductor wherein each of the charge transport layers, especially a first and second charge transport layer, comprises



wherein X is selected from the group consisting of lower, that is with, for example, from 1 to about 8 carbon atoms, alkyl, alkoxy, aryl, and halogen; a photoconductor wherein each, or at least one of the charge transport layers comprises



wherein X and Y are independently lower alkyl, lower alkoxy, phenyl, a halogen, or mixtures thereof, and wherein the photogenerating and charge transport layer resinous binder is selected from the group consisting of polycarbonates and polystyrene; a photoconductor wherein the photogenerating pigment present in the photogenerating layer is comprised of chlorogallium phthalocyanine, or Type V hydroxygallium phthalocyanine prepared by hydrolyzing a gallium phthalocyanine precursor by dissolving the hydroxygallium phthalocyanine in a strong acid, and then reprecipitating the resulting dissolved precursor in a basic aqueous media; removing any ionic species formed by washing with water; concentrating the resulting aqueous slurry comprised of water and hydroxygallium phthalocyanine to a wet cake; removing water from the wet cake by drying; and subjecting the resulting dry pigment to mixing with the addition of a second solvent to cause the formation of the hydroxygallium phthalocyanine; an imaging member wherein the Type V hydroxygallium phthalocyanine has major peaks, as measured with an X-ray diffractometer, at Bragg angles (2 theta+/-0.2°) 7.4,

9.8, 12.4, 16.2, 17.6, 18.4, 21.9, 23.9, 25.0, 28.1 degrees, and the highest peak at 7.4 degrees; a method of imaging which comprises generating an electrostatic latent image on the photoconductor developing the latent image, and transferring the developed electrostatic image to a suitable substrate; a method of imaging wherein the imaging member is exposed to light of a wavelength of from about 370 to about 950 nanometers; a member wherein the photogenerating layer is of a thickness of from about 0.1 to about 50 microns; a member wherein the photogenerating pigment is dispersed in from about 1 weight percent to about 80 weight percent of a polymer binder; a member wherein the binder is present in an amount of from about 50 to about 90 percent by weight, and wherein the total of the layer components is about 100 percent; a photoconductor wherein the photogenerating component is Type V hydroxygallium phthalocyanine, or chlorogallium phthalocyanine, and the charge transport layer contains a hole transport of N,N'-diphenyl-N,N-bis(3-methylphenyl)-1,1'-biphenyl-4,4'-diamine, N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis-(4-isopropylphenyl)-[p-terphenyl]-4,4"-diamine, N,N'-bis(4-butylphenyl)-N,N'-bis-(2-ethyl-6-methylphenyl)-[p-terphenyl]-4,4"-diamine, N,N'-bis(4-butylphenyl)-N,N'-bis-(2,5-dimethylphenyl)-[p-terphenyl]-4,4"-diamine, N,N'-diphenyl-N,N'-bis(3-chlorophenyl)-[p-terphenyl]-4,4"-diamine molecules, and wherein the hole transport resinous binder is selected from the group consisting of polycarbonates and polystyrene; an imaging member wherein the photogenerating layer contains a metal free phthalocyanine; a photoconductive imaging member comprised of a supporting substrate, a doped photogenerating layer, a hole transport layer, and in embodiments wherein a plurality of charge transport layers are selected, such as for example, from two to about ten, and more specifically two, may be selected; and a photoconductive imaging member comprised of an optional supporting substrate, a photogenerating layer, and a first, second, and third charge transport layer.

The following Examples are being submitted to illustrate embodiments of the present disclosure.

#### COMPARATIVE EXAMPLE 1

There was prepared a photoconductor with a biaxially oriented polyethylene naphthalate substrate (KALEDEX™ 2000) having a thickness of 3.5 mils, and thereover, a 0.02 micron thick titanium layer was coated on the biaxially oriented polyethylene naphthalate substrate (KALEDEX™ 2000). Subsequently, there was applied thereon, with a gravure applicator or an extrusion coater, a hole blocking layer solution containing 50 grams of 3-aminopropyl triethoxysilane ( $\gamma$ -APS), 41.2 grams of water, 15 grams of acetic acid, 684.8 grams of denatured alcohol, and 200 grams of heptane. This layer was then dried for about 1 minute at 120° C. in a forced air dryer. The resulting hole blocking layer had a dry thickness of 500 Angstroms. An adhesive layer was then deposited by applying a wet coating over the blocking layer, using a gravure applicator or an extrusion coater, and which adhesive contained 0.2 percent by weight based on the total weight of the solution of the copolyester adhesive (ARDEL D100™ available from Toyota Hsutsu Inc.) in a 60:30:10 volume ratio mixture of tetrahydrofuran/monochlorobenzene/methylene chloride. The adhesive layer was then dried

for about 1 minute at 120° C. in the forced air dryer of the coater. The resulting adhesive layer had a dry thickness of 200 Angstroms.

A photogenerating layer dispersion was prepared by introducing 0.45 gram of the known polycarbonate IUPILON 200<sup>TM</sup> (PCZ-200) weight average molecular weight of 20,000, available from Mitsubishi Gas Chemical Corporation, and 50 milliliters of tetrahydrofuran into a 4 ounce glass bottle. To this solution were added 2.4 grams of hydroxygallium phthalocyanine (Type V) and 300 grams of 1/8 inch (3.2 millimeters) diameter stainless steel shot. This mixture was then placed on a ball mill for 8 hours. Subsequently, 2.25 grams of PCZ-200 were dissolved in 46.1 grams of tetrahydrofuran, and added to the hydroxygallium phthalocyanine dispersion. This slurry was then placed on a shaker for 10 minutes. The resulting dispersion was, thereafter, applied to the above adhesive interface with a Bird applicator to form a photogenerating layer having a wet thickness of 0.25 mil. A strip about 10 millimeters wide along one edge of the substrate web bearing the blocking layer and the adhesive layer was deliberately left uncoated by any of the photogenerating layer material to facilitate adequate electrical contact by the ground strip layer that was applied later. The photogenerating layer was dried at 120° C. for 1 minute in a forced air oven to form a dry photogenerating layer having a thickness of 0.4 micron.

The resulting photoconductor web was then coated with a dual charge transport layer. The first charge transport layer was prepared by introducing into an amber glass bottle in a weight ratio of 50/50, N,N'-bis(methylphenyl)-1,1-biphenyl-4,4'-diamine (TBD) and poly(4,4'-isopropylidene diphenyl) carbonate, a known bisphenol A polycarbonate having a  $M_w$  molecular weight average of about 120,000, commercially available from Farbenfabriken Bayer A.G. as MAKROLON<sup>®</sup> 5705. The resulting mixture was then dissolved in methylene chloride to form a solution containing 15.6 percent by weight solids. This solution was applied on the photogenerating layer to form the charge transport layer coating that upon drying (120° C. for 1 minute) had a thickness of 16.5 microns. During this coating process, the humidity was equal to or less than 30 percent, for example 25 percent.

The above first pass charge transport layer (CTL) was then overcoated with a second top charge transport layer in a second pass. The charge transport layer solution of the top layer was prepared introducing into an amber glass bottle in a weight ratio of 35/65, N,N'-bis(methylphenyl)-1,1-biphenyl-4,4'-diamine (TBD) and poly(4,4'-isopropylidene diphenyl) carbonate, a known bisphenol A polycarbonate having a  $M_w$  molecular weight average of about 120,000, commercially available from Farbenfabriken Bayer A.G. as MAKROLON<sup>®</sup> 5705. The resulting mixture was then dissolved in methylene chloride to form a solution containing 15.6 percent by weight solids. This solution was applied, using a 2 mil Bird bar, on the bottom layer of the charge transport layer to form a coating that upon drying (120° C. for 1 minute) had a thickness of 16.5 microns. During this coating process, the humidity was equal to or less than 15 percent. The total two-layer CTL thickness was 33 microns.

#### EXAMPLE I

A photoconductor was prepared by repeating the process of Comparative Example 1 except that there was included in the first pass charge transport layer 40 parts per million (0.004 percent by weight) of the additive triisobutyl(methyl)phosphonium tosylate (CYPHOS<sup>®</sup> IL 106, available from CYTEC), which tosylate salt was added to and mixed with the

above prepared first pass charge transport layer solution prior to the coating thereof on the photogenerating layer. More specifically, the triisobutyl(methyl)phosphonium tosylate additive was first dissolved in the charge transport layer solvent of methylene chloride, and then the resulting mixture was mixed with the above charge transport components of 50/50, N,N'-bis(methylphenyl)-1,1-biphenyl-4,4'-diamine and poly(4,4'-isopropylidene diphenyl) carbonate, a known bisphenol A polycarbonate having a  $M_w$  molecular weight average of about 120,000, commercially available from Farbenfabriken Bayer A.G. as MAKROLON<sup>®</sup> 5705. Thereafter, the mixture resulting was deposited on the photogenerating layer to form the first charge transport additive layer.

#### EXAMPLE II

A photoconductor is prepared by repeating the process of Example I except that there is included in the first pass charge transport layer 100 parts per million (0.01 percent by weight) of the additive tetradecyl(triethyl)phosphonium dicyanamide (CYPHOS<sup>®</sup> IL 105, available from CYTEC).

#### EXAMPLE III

A photoconductor is prepared by repeating the process of Example I except that there is included in the first pass charge transport layer 500 parts per million (0.05 percent by weight) of the additive tetradecyl(triethyl)phosphonium bis triflimate (CYPHOS<sup>®</sup> IL 109, available from CYTEC).

#### EXAMPLE IV

A photoconductor is prepared by repeating the process of Example I except that there is included in the first pass charge transport layer 200 parts per million (0.02 percent by weight) of the additive tetradecyl(triethyl)phosphonium chloride.

#### EXAMPLE V

A photoconductor is prepared by repeating the process of Example I except that there is included in the first pass charge transport layer 200 parts per million (0.02 percent by weight) of the additive 4-(carboxybutyl)triphenylphosphonium bromide.

#### EXAMPLE VI

A photoconductor is prepared by repeating the process of Example I except that there is included in the first pass charge transport layer 200 parts per million (0.02 percent by weight) of the additive tetrabutylphosphonium benzotriazolate.

#### Electrical Property Testing

The above prepared photoconductors of Comparative Example 1 and Example I were tested in a scanner set to obtain photoinduced discharge cycles, sequenced at one charge-erase cycle followed by one charge-expose-erase cycle, wherein the light intensity was incrementally increased with cycling to produce a series of photoinduced discharge characteristic curves from which the photosensitivity and surface potentials at various exposure intensities were measured. Additional electrical characteristics were obtained by a series of charge-erase cycles with incrementing surface potential to generate several voltage versus charge density curves. The scanner was equipped with a scorotron set to a constant voltage charging at various surface potentials. The

devices were tested at surface potentials of 400 volts with the exposure light intensity incrementally increased by means of regulating a series of neutral density filters; and the exposure light source was a 780 nanometer light emitting diode. The xerographic simulation was completed in an environmentally controlled light tight chamber at ambient conditions (40 percent relative humidity and 22° C.).

The results are summarized in Table 1 wherein  $dV/dX$  (in  $V/cm^2/erg$ ) is the photosensitivity as determined by the initial slope of the photoinduced discharge curve plotted as surface potential (in volts) versus exposure energy (in  $erg/cm^2$ ),  $V(2.2)$  is the surface potential of the photoreceptors or photoconductors at an exposure energy of 2.2  $ergs/cm^2$ , and  $V_{erase}$  is the surface potential of the photoconductors after they were subjected to an erase light of 680 nanometers at an intensity of about 100 to 150  $erg s/cm^2$ .

TABLE 1

|             | $dV/dX$ ( $V/cm^2/erg$ ) | $V(2.2)$ (V) | $V_{erase}$ (V) |
|-------------|--------------------------|--------------|-----------------|
| Comparative | -478                     | 77           | 42              |
| Example 1   | -440                     | 106          | 69              |
| Example I   |                          |              |                 |

With incorporation of the phosphonium salt in the first pass charge transport layer, the PIDC was tuned to a slower value with decreased photosensitivity, and increased  $V(2.2)$  and  $V_{erase}$ . For example, with 40 ppm of the salt in the first pass charge transport layer (Example I), the photosensitivity was decreased by about 8 percent, and the  $V(2.2)$  was increased by about 30V (volts).

Thus, the incorporation of the phosphonium salt can effectively adjust the PIDC, thus providing, for example, a feasible approach for on-line tuning of the photoconductor PIDC to achieve excellent photoconductor production or manufacturing yields. In production, the additive can be added into the first pass charge transport layer solution when the on-line PIDC output is fast (higher photosensitivity and lower  $V(2.2)$ ), thus adjusting the PIDC characteristics and preventing or minimizing a loss in yields.

#### Charge Deficient Spots (CDS) Measurement

Various known methods have been developed to assess and/or accommodate the occurrence of charge deficient spots. For example, U.S. Pat. Nos. 5,703,487 and 6,008,653, the disclosures of each patent being totally incorporated herein by reference, disclose processes for ascertaining the micro-defect levels of an electrophotographic imaging member or photoconductor. The method of U.S. Pat. No. 5,703,487, designated as field-induced dark decay (FIDD), involves measuring either the differential increase in charge over and above the capacitive value, or measuring reduction in voltage below the capacitive value of a known imaging member and of a virgin imaging member, and comparing differential increase in charge over and above the capacitive value or the reduction in voltage below the capacitive value of the known imaging member and of the virgin imaging member.

U.S. Pat. Nos. 6,008,653 and 6,150,824, the disclosures of each patent being totally incorporated herein by reference, disclose a method for detecting surface potential charge patterns in an electrophotographic imaging member with a floating probe scanner. Floating Probe Micro Defect Scanner (FPS) is a contactless process for detecting surface potential charge patterns in an electrophotographic imaging member. The scanner includes a capacitive probe having an outer

shield electrode, which maintains the probe adjacent to and spaced from the imaging surface to form a parallel plate capacitor with a gas between the probe and the imaging surface, a probe amplifier optically coupled to the probe, establishing relative movement between the probe and the imaging surface, and a floating fixture which maintains a substantially constant distance between the probe and the imaging surface. A constant voltage charge is applied to the imaging surface prior to relative movement of the probe and the imaging surface past each other, and the probe is synchronously biased to within about  $\pm 300$  volts of the average surface potential of the imaging surface to prevent breakdown, measuring variations in surface potential with the probe, compensating the surface potential variations for variations in distance between the probe and the imaging surface, and comparing the compensated voltage values to a baseline voltage value to detect charge patterns in the electrophotographic imaging member. This process may be conducted with a contactless scanning system comprising a high resolution capacitive probe, a low spatial resolution electrostatic voltmeter coupled to a bias voltage amplifier, and an imaging member having an imaging surface capacitively coupled to and spaced from the probe and the voltmeter. The probe comprises an inner electrode surrounded by and insulated from a coaxial outer Faraday shield electrode, the inner electrode connected to an opto-coupled amplifier, and the Faraday shield connected to the bias voltage amplifier. A threshold of 20 volts is commonly chosen to count charge deficient spots. A number of the above prepared photoconductors were measured for CDS counts using the above-described FPS technique, and the results follow in Table 2.

TABLE 2

|                       | CDS (Counts/cm <sup>2</sup> ) |
|-----------------------|-------------------------------|
| Comparative Example 1 | 5.2                           |
| Example I             | 4.9                           |

There were no detrimental effects on CDS when 40 parts per million concentration of the salt was incorporated into the first charge transport layer.

The claims, as originally presented and as they may be amended, encompass variations, alternatives, modifications, improvements, equivalents, and substantial equivalents of the embodiments and teachings disclosed herein, including those that are presently unforeseen or unappreciated, and that, for example, may arise from applicants/patentees and others. Unless specifically recited in a claim, steps or components of claims should not be implied or imported from the specification or any other claims as to any particular order, number, position, size, shape, angle, color, or material.

What is claimed is:

1. A photoconductor comprising a supporting substrate, a photogenerating layer, and at least one charge transport layer comprised of at least one charge transport component, and wherein said at least one charge transport layer contains at least one phosphonium salt, and wherein said salt is present in an amount of from about 0.0001 to about 2.5 weight percent.
2. A photoconductor in accordance with claim 1 wherein said salt is an alkyl phosphonium salt.
3. A photoconductor in accordance with claim 2 wherein said alkyl contains from 1 to about 18 carbon atoms.
4. A photoconductor in accordance with claim 1 wherein said salt is triisobutyl(methyl)phosphonium tosylate.
5. A photoconductor in accordance with claim 1 wherein said salt is at least one of tetradecyl(trihexyl)phosphonium

31

chloride, tetradecyl(trihexyl)phosphonium decanoate, trihexyl(tetradecyl)phosphonium bis 2,4,4-trimethylpentyl phosphinate, tetradecyl(trihexyl)phosphonium dicyanamide, tetradecyl(trihexyl)phosphonium bistriflamide, tetradecyl(trihexyl)phosphonium hexafluorophosphate, tetradecyl(trihexyl)phosphonium tetrafluoroborate, ethyl tri(butyl)phosphonium diethylphosphate, (N-methyl-N-phenylamino)triphenylphosphonium iodide, 2-dimethylaminoethyltriphenylphosphonium bromide, 4-(carboxybutyl)triphenyl phosphonium bromide, amyltriphenylphosphonium bromide, tetrabutylphosphonium benzotriazolate, tetrabutylphosphonium tetraphenylborate, tetrakis(hydroxymethyl)phosphonium chloride, and tributylmethylphosphonium iodide.

6. A photoconductor in accordance with claim 1 wherein said salt is present in an amount of from about 20 parts per million to about 500 parts per million.

7. A photoconductor in accordance with claim 1 wherein said salt is present in an amount of from about 40 parts per million to about 300 parts per million.

8. A photoconductor in accordance with claim 1 wherein said salt is triisobutyl(ethyl)phosphonium tosylate, tetradecyl(trihexyl)phosphonium dicyanamide, or tetradecyl(trihexyl)phosphonium bistriflamide present in an amount of from about 10 parts per million to about 200 parts per million.

9. A photoconductor in accordance with claim 1 wherein said charge transport component is comprised of at least one of aryl amine molecules



wherein X is selected from the group consisting of at least one of alkyl, alkoxy, aryl, and halogen; and wherein X, Y and Z are independently selected from the group consisting of at least one of alkyl, alkoxy, aryl, and halogen.

10. A photoconductor in accordance with claim 1 wherein said charge transport component is an aryl amine selected from the group consisting of N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis-(4-isopropylphenyl)-[p-

32

terphenyl]-4,4"-diamine, N,N'-bis(4-butylphenyl)-N,N'-bis(2-ethyl-6-methylphenyl)-[p-terphenyl]-4,4"-diamine, N,N'-bis(4-butylphenyl)-N,N'-bis-(2,5-dimethylphenyl)-[p-terphenyl]-4,4"-diamine, N,N'-diphenyl-N,N'-bis(3-chlorophenyl)-[p-terphenyl]-4,4"-diamine, and mixtures thereof, and wherein said at least one charge transport layer is from 1 to about 4, and wherein said salt is tetradecyl(trihexyl)phosphonium chloride, tetradecyl(trihexyl)phosphonium decanoate, trihexyl(tetradecyl)phosphonium bis 2,4,4-trimethylpentylphosphinate, tetradecyl(trihexyl)phosphonium dicyanamide, triisobutyl(methyl)phosphonium tosylate, tetradecyl(trihexyl)phosphonium bistriflamide, tetradecyl(trihexyl)phosphonium hexafluorophosphate, tetradecyl(trihexyl)phosphonium tetrafluoroborate, ethyl tri(butyl)phosphonium diethylphosphate, (N-methyl-N-phenylamino)triphenylphosphonium iodide, 2-dimethylaminoethyltriphenyl phosphonium bromide, 4-(carboxybutyl)triphenylphosphonium bromide, amyltriphenylphosphonium bromide, tetrabutylphosphonium benzotriazolate, tetrabutylphosphonium tetraphenylborate, tetrakis(hydroxymethyl)phosphonium chloride, and tributylmethylphosphonium iodide.

11. A photoconductor in accordance with claim 1 further including in at least one of said charge transport layers an antioxidant comprised of at least one of a hindered phenolic and a hindered amine, and wherein said at least one charge transport layer is from 1 to about 4.

12. A photoconductor in accordance with claim 1 wherein said photogenerating layer is comprised of at least one photogenerating pigment.

13. A photoconductor in accordance with claim 12 wherein said photogenerating pigment is comprised of at least one of a metal phthalocyanine, a perylene, and a metal free phthalocyanine.

14. A photoconductor in accordance with claim 12 wherein said photogenerating pigment is comprised of chlorogallium phthalocyanine, or a titanyl phthalocyanine.

15. A photoconductor in accordance with claim 12 wherein said photogenerating pigment is comprised of hydroxygallium phthalocyanine.

16. A photoconductor in accordance with claim 1 further including a hole blocking layer, and an adhesive layer.

17. A photoconductor in accordance with claim 1 wherein said at least one charge transport layer is comprised of a first and a second charge transport layer, and wherein said salt is included in said first charge transport layer in an amount of from about 20 to about 175 parts per million based on the first charge transport layer components.

18. A photoconductor in accordance with claim 1 wherein said at least one charge transport layer is comprised of a top charge transport layer and a bottom charge transport layer, and wherein said top layer is in contact with said bottom layer and said bottom layer is in contact with said photogenerating layer, and wherein said bottom layer includes a salt of tetradecyl(trihexyl)phosphonium chloride, tetradecyl(trihexyl)phosphonium decanoate, trihexyl(tetradecyl)phosphonium bis 2,4,4-trimethylpentylphosphinate, tetradecyl(trihexyl)phosphonium dicyanamide, triisobutyl(methyl)phosphonium tosylate, tetradecyl(trihexyl)phosphonium bistriflamide, tetradecyl(trihexyl)phosphonium hexafluorophosphate, tetradecyl(trihexyl)phosphonium tetrafluoroborate, ethyl tri(butyl)phosphonium diethylphosphate, (N-methyl-N-phenylamino)triphenylphosphonium iodide, 2-dimethylaminoethyltriphenylphosphonium bromide, 4-(carboxybutyl)triphenyl phosphonium bromide, amyltriphenylphosphonium bromide, tetrabutylphosphonium benzotriazolate, tetrabutylphosphonium tetraphenylborate,

60 tetradecyl(trihexyl)phosphonium chloride, tetradecyl(trihexyl)phosphonium decanoate, trihexyl(tetradecyl)phosphonium bis 2,4,4-trimethylpentylphosphinate, tetradecyl(trihexyl)phosphonium dicyanamide, triisobutyl(methyl)phosphonium tosylate, tetradecyl(trihexyl)phosphonium bistriflamide, tetradecyl(trihexyl)phosphonium hexafluorophosphate, tetradecyl(trihexyl)phosphonium tetrafluoroborate, ethyl tri(butyl)phosphonium diethylphosphate, (N-methyl-N-phenylamino)triphenylphosphonium iodide, 2-dimethylaminoethyltriphenylphosphonium bromide, 4-(carboxybutyl)triphenylphosphonium bromide, amyltriphenylphosphonium bromide, tetrabutylphosphonium benzotriazolate, tetrabutylphosphonium tetraphenylborate,

33

rate, tetrakis(hydroxymethyl)phosphonium chloride, or tributylmethylphosphonium iodide.

**19.** A photoconductor comprised in sequence of a supporting substrate, a photogenerating layer, and a charge transport layer; and wherein said charge transport layer contains a phosphonium salt.

**20.** A photoconductor in accordance with claim **19** wherein said charge transport layer is comprised of a first charge transport layer and a second charge transport layer, and wherein said salt is included in said first charge transport layer in contact with said photogenerating layer, and said salt is present in an amount of from about 10 parts per million to about 500 parts per million.

**21.** A photoconductor in accordance with claim **20** wherein said salt is at least one of tetradecyl(triethyl)phosphonium chloride, tetradecyl(triethyl) phosphonium decanoate, trihexyl(tetradecyl)phosphonium bis 2,4,4-trimethylpentylphosphinate, tetradecyl(triethyl)phosphonium dicyanamide, triisobutyl(methyl)phosphonium tosylate, tetradecyl (triethyl)phosphonium bistriflamide, tetradecyl(triethyl) phosphonium hexafluorophosphate, tetradecyl(triethyl) phosphonium tetrafluoroborate, ethyl tri(butyl)phosphonium diethylphosphate, (N-methyl-N-phenylamino)triphenylphosphonium iodide, 2-dimethylaminoethyltriphenylphosphonium bromide, 4-(carboxybutyl)triphenyl phosphonium bromide, amyltriphenylphosphonium bromide, tetrabutylphosphonium benzotriazolate, tetrabutylphosphonium tetraphenylborate, tetrakis(hydroxymethyl)phosphonium chloride, and tributylmethylphosphonium iodide, and which salt is present in an amount of from about 0.003 to about 3 weight percent.

34

**22.** A photoconductor in accordance with claim **1** wherein the substrate is comprised of aluminum, wherein said salt primarily functions to control the photosensitivity of said photoconductor, and wherein said salt is present in an amount of from about 0.001 to about 1 weight percent.

**23.** A photoconductor comprising a supporting substrate, a photogenerating layer, a first hole transport layer and a second hole transport layer, and wherein said first hole transport layer has incorporated therein a phosphonium salt selected from the group consisting of tetradecyl(triethyl)phosphonium chloride, tetradecyl(triethyl)phosphonium decanoate, trihexyl(tetradecyl)phosphonium bis 2,4,4-trimethylpentylphosphinate, tetradecyl(triethyl)phosphonium dicyanamide, triisobutyl(methyl)phosphonium tosylate, tetradecyl (triethyl)phosphonium bistriflamide, tetradecyl(triethyl) phosphonium hexafluorophosphate, tetradecyl(triethyl) phosphonium tetrafluoroborate, ethyl tri(butyl)phosphonium diethylphosphate, (N-methyl-N-phenylamino)triphenylphosphonium iodide, 2-dimethylaminoethyltriphenylphosphonium bromide, 4-(carboxybutyl)triphenyl phosphonium bromide, amyltriphenylphosphonium bromide, tetrabutylphosphonium benzotriazolate, tetrabutylphosphonium tetraphenylborate, tetrakis(hydroxymethyl) phosphonium chloride, tributylmethylphosphonium iodide, and mixtures thereof, and which salt is present in an amount of from about 2 to about 300 parts per million.

**24.** A photoconductor in accordance with claim **23** wherein said salt is triisobutyl(methyl)phosphonium tosylate.

\* \* \* \* \*